

## UNITED STATES PATENT OFFICE

2,425,174

## LUBRICANT COMPOSITION

Emmett S. Carmichael, Jackson Heights, and  
 Theodore G. Roehner, Malverne, N. Y., as-  
 signors to Socony-Vacuum Oil Company, In-  
 corporated, New York, N. Y., a corporation of  
 New York

No Drawing. Application July 31, 1941,  
 Serial No. 404,840

8 Claims. (Cl. 252—33)

1

This invention relates to a lubricant for cold rolling of steel, particularly thin gauge metal such as that destined for tin plate.

Soluble oil emulsions have long been used for rolling steel where reductions to gauge were small and where the surface structure of the metal was not as important as for tin plate. Aqueous roll lubricants for this application have been emulsions of the oil-in-water type, and their principal value has been as coolants. Experience has shown that emulsions of the oil-in-water type remain completely ineffective as lubricants for rolling tin plate for a period of 36 to 48 hours, and only after such "break in" period begin to show a lubricating value. Spoilage and loss of steel during this "break in" period is large, the rate of production is low, and general dissatisfaction exists among the rollers in the mills because of the adverse effect on the equipment and production.

As an example of such commercially used roll lubricants we give the following:

|                     | Per cent |
|---------------------|----------|
| Palm oil            | 50       |
| Mineral soluble oil | 50       |

A 1 to 9 emulsion is prepared by mixing the above lubricant with water. This oil-in-water emulsion is fed to the roll stands.

This invention has for its object the provision of an emulsion type of rolling lubricant which is immediately effective upon application. A further object is the provision of a lubricant of novel compound emulsion characteristics.

We have made the discovery that if a roll lubricant capable of forming an oil-in-water emulsion is treated with a small amount of mineral salt of metals or any other bases inorganic or organic, capable of reversing the phases of the emulsion, the resulting compound emulsion is suitable for immediate application without any undesirable "breaking in" period. While the mechanism of the lubrication is not exactly known, it is the belief of the inventors that the success of their discovery can be attributed to the fact that a compound emulsion is formed. By that is meant that a water-in-oil emulsion of the roll lubricant is dispersed in the balance of the water thus forming three phases: water-oil-water.

As an example of roll lubricant representative of this invention, we give the following:

2

## Example I

|                     |                    |      |
|---------------------|--------------------|------|
| Palm oil            | per cent by weight | 4.9  |
| Mineral soluble oil | do                 | 4.9  |
| Magnesium sulfate   | per cent           | .2   |
| Water               | do                 | 90.0 |

The procedure for the preparation of the emulsified roll lubricant is as follows: Equal parts of palm oil and mineral soluble oil are mixed with almost the total quantity of water. Unless the palm oil contains excessive quantities of free fatty acids, an oil-in-water emulsion is easily formed. To that emulsion the solution of magnesium sulfate in the balance of the water, as shown in the formula, is added, thus forming the compound emulsion.

An excess of free fatty acids in the palm oil may prevent the emulsification of the mixture of palm oil and soluble oil. In this case the soluble oil is first emulsified with almost the total amount of water; then the palm oil is added gradually with agitation and finally the solution of magnesium sulfate is stirred in.

The characterizing ingredients of the presently discussed composition are a soluble oil capable of forming an oil-in-water emulsion, and an emulsion inverting material, so handled as to form a three phase dispersion system in which an oil-external-water-internal dispersion is itself dispersed to form the internal phase in an aqueous emulsion.

The oleaginous or soluble oil material is composed of an oil or oil mixture and an emulsifier capable of forming an oil-in-water emulsion. The oily material may be wholly mineral oil, although such compositions are relatively less effectual, but is preferably composed substantially of a vegetable or animal oil or fat, such as palm oil, cocoanut oil, cottonseed oil, wool fat, lard oil, tallow, fish oil, hydrogenated fatty oils, and the like.

The emulsifier capable of forming oil-in-water emulsions, which is compounded with the oily material to form a soluble oil may be any of the usual emulsifiers so used. A very typical and usual material of this type is an alkali soap of a mineral oil sulphonate, with or without assistant emulsifying agents. The emulsifier mixture of the example designated herein as "mineral soluble oil" was a mixture of oil, the sodium soaps of

mineral oil sulphonates, and potassium salts of the fatty acids frequently designated as "tall oil" and derived from sulphite paper pulp mill waste. Numerous other common emulsifying agents may be so used such as alkali soaps of rosin, oleic acid, naphthenic acids, etc.

The emulsion inverter material may be any one of those numerous salts of bivalent or polyvalent metals or organic bases which are capable of inverting oil-in-water emulsions to form water-in-oil emulsions. Magnesium sulphate is a cheap and effective material which commonly is so used. Other such materials are calcium chloride, zinc chloride, lead chloride, the chlorides of iron, aluminum sulfate, diglycol stearate, glycol oleate, etc.

It will be remembered that the lubricating composition has been described as a water-in-oil-in-water compound emulsion. Its unusual properties are coupled with the attainment and maintenance of this structure. Too much of either the emulsifier material or of the emulsion inverter material will cause the mixture to pass over either to an oil-in-water or a water-in-oil emulsion, neither of which is effective. To this end, proportioning of the materials used must be definitely controlled.

No general rule for the proportioning of the emulsion-inverter can be given in terms of numerical values, for the optimum quantity of the inverter to be used in any given formulation is dependent upon such factors as the quantity and nature of the soaps used, the free acidity, etc. Consequently the amount must be determined by experiment, in the usual manner, with each formulation. For the particular formulation given in Example I above, using magnesium sulphate as inverter, the amount of inverter should be less than 0.5% and preferably between 0.1% and 0.3%.

We claim:

1. A lubricant for use in the cold rolling of steel comprising an emulsion wherein water is the continuous phase and the disperse phase is a water-in-oil emulsion, said composition being constituted of water, a lubricating oleaginous material, an emulsifier capable of emulsifying the oleaginous material in water, and sufficient amount of a salt of a polyvalent metal to bring about the formation of an emulsion of the compound type.

2. A lubricant composition comprising a lubricating oleaginous material selected from the group consisting of mineral oils, animal oils and vegetable oils and mixtures thereof, a surface active material to emulsify the oleaginous material in water, water, and a material selected from the group consisting of salts of polyvalent metals capable of causing phase inversion of the first formed emulsion, the water, lubricant, emulsifier, and inverter being present in such proportions as to give a stable water-continuous emulsion the oil droplets of which are themselves a water-in-oil emulsion.

3. A lubricant for cold rolling metal comprising a lubricating oleaginous material selected from the group mineral oils, animal oils, vegetable oils, and mixtures thereof, which oleaginous material is dispersed as the internal phase of an oil-in-water emulsion, and which itself is the external phase of a water-in-oil emulsion, an emulsifier capable of emulsifying said oleaginous material in water, and a phase inverter selected from the group consisting of esters of polyvalent organic bases capable of inverting oil-in-water emulsions, the water, lubricant, emulsifier, and inverter being present in such proportions as to give a stable water-continuous emulsion the oil droplets of which are themselves a water-in-oil emulsion.

inverter being present in such proportions as to give a stable water-continuous emulsion the oil droplets of which are themselves a water-in-oil emulsion.

5. A lubricant composition comprising water, a lubricating oleaginous material selected from the group consisting of mineral oils, animal oils, vegetable oils and mixtures thereof, a surface active material selected from the group consisting of alkali soaps of rosin, oleic acid, sulphonic acids, naphthenic acids, and heavy fatty acids, and a phase inverter selected from the group consisting of magnesium sulphate, calcium chloride, lead chloride, zinc chloride, iron chlorides, aluminum sulphate; the emulsifier and phase inverter being so proportioned as to give rise to water-in-oil emulsion particles dispersed in a continuous water phase.

6. A method of lubricating steel subjected to gauge reduction in cold rolling by applying to the steel being rolled a lubricant comprising an emulsion wherein water is the continuous phase and the disperse phase is a water-in-oil emulsion, said composition being constituted of water, a lubricating oleaginous material, an emulsifier capable of emulsifying the oleaginous material in water, and a sufficient amount of an emulsion inverter, to effect the formation of an emulsion of the compound type.

7. A method of lubricating steel subjected to gauge reduction in cold rolling by applying to the steel being rolled a lubricant comprising a lubricating oleaginous material selected from the group consisting of mineral oil, animal oils and vegetable oils and mixtures thereof, a surface active material to emulsify the oleaginous material in water, water, and a material selected from the group consisting of salts of polyvalent metals capable of causing phase inversion of the first formed emulsion, the water, lubricant, emulsifier, and inverter being present in such proportions as to give a stable water-continuous emulsion the oil droplets of which are themselves a water-in-oil emulsion.

8. A method of lubricating steel subjected to gauge reduction in cold rolling by applying to the steel being rolled a lubricant comprising a lubricating oleaginous material selected from the group mineral oils, animal oils, vegetable oils, and mixtures thereof, which oleaginous material is dispersed as the internal phase of an oil-in-water emulsion, and which itself is the external phase of a water-in-oil emulsion, an emulsifier capable of emulsifying said oleaginous material in water, and a phase inverter selected from the group consisting of esters of polyvalent organic bases capable of inverting oil-in-water emulsions, the water, lubricant, emulsifier, and inverter being present in such proportions as to give a stable water-continuous emulsion the oil droplets of which are themselves a water-in-oil emulsion.

9. A method of lubricating steel subjected to gauge reduction in cold rolling by applying to the steel being rolled a lubricant comprising water, a lubricating oleaginous material selected from the group consisting of mineral oils, animal oils, vegetable oils and mixtures thereof, a surface active material selected from the group consisting of alkali soaps of rosin, oleic acid, sulphonic acids, naphthenic acids, and heavy fatty acids, and a phase inverter selected from the group consisting of magnesium sulphate, calcium chloride, lead chloride, zinc chloride, iron chlorides, aluminum sulphate; the emulsifier and

phase inverter being so proportioned as to give rise to water-in-oil emulsion particles dispersed in a continuous water phase.

EMMETT S. CARMICHAEL  
THEODORE G. ROEHNER.

## REFERENCES CITED

The following references are of record in the file of this patent:

## UNITED STATES PATENTS

| Number    | Name     | Date          |
|-----------|----------|---------------|
| 2,071,488 | Zimmer   | Feb. 23, 1937 |
| 2,152,396 | Williams | Mar. 28, 1939 |

| Number    | Name       | Date           |
|-----------|------------|----------------|
| 2,231,214 | Nelson     | Feb. 11, 1941  |
| 2,307,744 | Liberthson | Jan. 12, 1943  |
| 2,303,142 | Spangler   | Nov. 24, 1942  |
| 2,230,556 | Zimmer     | Feb. 4, 1941   |
| 2,214,634 | Dombrow    | Sept. 10, 1940 |
| 1,724,653 | Hertman    | Aug. 13, 1939  |

## OTHER REFERENCES

- 10 Phase Volume Theory and the Homogenization of Concentrated Emulsions, part II, by Parke, in Journal of the Chemical Society of London, pages 1112-1115, pt. 2, July-Dec. 1934 Proceed. Studies in Emulsions, by Seifriz, in Journal of Physical Chemistry, vol. 29, 1925, pages 738-749.